

Nov. 17, 1925.

1,562,385

C. M. TAYLOR

FLOOR COVERING AND PROCESS OF MAKING SAME

Original Filed Jan. 10, 1922

FIG. 1.



FIG. 2.



Inventor

C. Marshall Taylor

By Prentiss, Stone & Boyden  
Attorneys

## UNITED STATES PATENT OFFICE.

CALEB MARSHALL TAYLOR, OF ELIZABETH, NEW JERSEY.

## FLOOR COVERING AND PROCESS OF MAKING SAME.

Application filed January 10, 1922, Serial No. 528,301. Renewed September 1, 1925.

*To all whom it may concern:*

Be it known that I, CALEB MARSHALL TAYLOR, a citizen of the United States, residing at Elizabeth, in the county of Union 5 and State of New Jersey, have invented certain new and useful Improvements in Floor Coverings and Processes of Making Same, of which the following is a specification.

This invention relates to floor coverings 10 and to a process of making the same.

The floor covering provided is of that type known as felt base floor coverings and particularly such materials in which an asphalt or bitumen impregnated base is used.

15 The invention is also peculiarly adapted for use in combination with all floor coverings in which either the wear surface or the opposite face is formed of paint or other material containing linseed oil or other oil, 20 or any material subject to saponification or removable under the action of soap and the usual floor cleaning materials.

25 Bitumen impregnated felt base floor coverings may be recognized by the main dark body which is particularly evident when the material is cut. The felt of such bases may be made from rags or from paper or any cellulose material, or from a mixture of such material, thoroughly impregnated with 30 asphalt or tar or some suitable bituminous material. When used as a supporting base for floor covering it is the usual practice to coat the bitumen impregnated base with a layer of paint which is known as a sealing coat and often to apply various painted designs, all of which may be applied in any 35 convenient manner. Also, a coat of paint is applied to the opposite or under surface of the impregnated base to cover the dark and unsightly bitumen impregnated base.

40 In using such bitumen impregnated bases it has been found that the wear paint and the decorative paint may become discolored due in part to the inherent nature of the bitumen of the base. Also in drying the paint coats it is necessary to dry at relatively low temperatures and for a correspondingly long period, often as long as four or five days. A higher temperature and more rapid 45 drying would tend to liquefy the bitumen and delay proper drying of the paint and also discolor the paint due to the release of materials from the base. Thus a baking temperature of 175° or more, such as is de-

sirable for treating the paint coats, is not 55 advisable in the usual drying of such coated bases.

After the present known product is completed it is usually necessary to place paper between adjacent surfaces when the material is rolled or stacked in layers to prevent the adjacent painted surfaces from adhering. It is well known that all such painted surfaces, and also that the material known 60 as linoleum is worn away by the use of soap and water because of saponification by such 65 cleaning materials on the oils in the paint and linoleum.

The present invention makes it possible to 70 use the relatively inexpensive bitumen impregnated felt base without discoloration of the wear or decorative paint coats, and results not only in reducing the time of drying the paint coats a much shorter length of 75 time; but makes it possible to use a higher drying temperature for the paint and to produce a more lasting finish on the painted 80 surface. Further, the present invention also provides a transparent, flexible and tough 85 wear coat over the surface of the paint coats, and provides a surface of non-saponifiable material which will resist the action 90 of soap and water.

In producing the impregnated felt base of 95 this invention, the usual rolls of felt may be used. These may have been previously impregnated with a bituminous material, or may have been saturated with the cellulose ester solution in accordance with the details 100 described and claimed in my copending application Serial No. 528297, filed January 10, 1922. Or the base may have been saturated with the particular compound described and claimed in my copending application Serial No. 538143, filed February 20, 1922, in which compound there is a mixture of linseed oil or vegetable drying oils, a drier such as borate of manganese, and resin, such as cumaron, or kauri, or camphor and the impregnated base dried in accordance 105 with the particular steps set forth in that application.

A solution is prepared of a mixture of nitrocellulose and a solvent therefor. Preferably the desired quantity of a semi-drying 110 or drying vegetable oil is added to the mixture as a softening medium. The solution is applied to one or both sides of the im-

pregnated base as a sealing coat by any well known coating process. The solution thus applied is quickly dried on the base. A suitable drying temperature is approximately 5 140° F. The impregnated base is thus provided with an impervious film, and may be used where an ordinary bitumen impregnated base would not have been acceptable before on account of the sticky, tar-like nature of its materials.

One or more paint coats are then applied and the structure baked to dry the paint and provide the desired wearing surface. The coating of impervious pyroxylin over 15 the felt base prevents any dark material from the base from discoloring the paint. An outer coating of a cellulose solution is then applied by dipping the painted base or by brushing the solution over the paint 20 coat, or by any suitable spreading means, and finally the cellulose coating is dried.

In the preparation of a cellulose solution for the sealing coat and for the outer coat other cellulose esters, such as acetyl cellulose, may be used instead of nitrocellulose.

One satisfactory mixture for the coating solution used for the sealing coat may be made by using 12 parts by weight of nitro cotton, and 88 parts by weight of a solvent 30 mixture which may be composed of 35 per cent of acetone oil and 65 per cent of such a diluent as solvent naphtha, xylol, toluol, or benzol. Any well known working formula may be used for combining such a 35 mixture of drying or semi-drying vegetable oil and nitro cotton. To such a mixture may be added 12 parts by weight of linseed oil or other semi-drying or drying vegetable oil.

40 One satisfactory solution for the outer wear coat may be made by using 10 parts by weight of nitro cotton, and 90 parts by weight of a solvent mixture which may be composed of 35 per cent of acetone oil and 45 65 per cent of such a diluent as solvent naphtha, xylol, toluol, or benzol. Any well known working formula may be used for combining such a mixture of drying or semi-drying vegetable oil and nitro cotton. To such a mixture may be added 10 parts by weight of linseed oil or other semi-drying 50 or drying vegetable oil.

In the accompanying drawing:—

55 Figure 1 illustrates an enlarged sectional view of a felt base 1 having an upper coating 2 of the pyroxylin solution and if desirable an under coating 3 of the same material. A paint coat 4 is applied on top of the surface 2 and an outer decorative paint coat is indicated at 5. An outer wear coat of transparent pyroxylin is indicated at 6.

Figure 2 is a plan view of the material 60 illustrated in Figure 1.

65 Both the bottom coat and the wear coat

serve to increase the tensile strength, and these coats do away with the need of spacing paper in the shipment of the materials, whether the material be rolled or stacked in layers. The wear coat and the bottom 70 coat possess good wearing qualities and are non-saponifiable.

To either one or all of the cellulose coatings may be added 12 parts by weight of resin, such as cumaron, or kauri, or camphor 75 or such other quantity as may be desirable. Likewise to any of the mixtures used in the cellulose coatings a pigment color in any desired shade and amount can be added. This results in a tinted film formed from 80 the solution, as contrasted with a plastic material, in which the same shade extends through the thickness of the film and gives an opaque effect, a feature which is new in such cellulose coatings, and particularly in 85 floor coverings. This is to be contrasted to the tinted pyroxylin plastics such as are applied by plastic working apparatus. Preferably the outer wear coating is substantially transparent if it is immediately 90 over a decorative paint coat.

I claim:

1. A floor covering comprising an impregnated felt base saturated throughout 95 with an impregnating material and dried, a first imperforate coating of a cellulose ester on said base, a coating of paint on said cellulose ester, and a second and transparent coating of a cellulose ester on the outer surface of said paint coat.

2. A floor covering comprising an impregnated felt base saturated throughout with an impregnating material and dried, 105 a first imperforate coating of a mixture of a cellulose ester and a softening medium on said base, a coating of paint on said first coating, and a second and transparent coating of a cellulose ester on the outer surface of said paint coat.

3. A floor covering comprising an impregnated felt base saturated throughout with an impregnating material and dried, 110 a first imperforate coating of a nitrocellulose material on said base, a coating of paint on said first coat, and a second and transparent coating of nitrocellulose on the outer surface of said paint coat.

4. A floor covering comprising an impregnated felt base saturated throughout with an impregnating material and dried, 120 a first imperforate coating of a mixture of nitrocellulose and a softening medium on said base, a coating of paint on said first coating, and a second and transparent coating of nitrocellulose on the outer surface 125 of said paint coat.

5. A floor covering comprising an impregnated felt base, a first imperforate coating of a cellulose ester on the opposite faces of said base, a coating of paint on said cellu- 130

lose ester, and a second and transparent coating of a cellulose ester on the outer surface of said paint coat.

6. A floor covering comprising an impregnated felt base, a first imperforate coating of a mixture of a cellulose ester and a softening medium on the opposite faces of said base, a coating of paint on said first coating, and a second and transparent coating of a cellulose ester on the outer surface of said paint coat.

7. A floor covering comprising an impregnated felt base, a first imperforate coating of a nitrocellulose material on the opposite faces of said base, a coating of paint on said first coat, and a second and transparent coating of nitrocellulose on the outer surface of said paint coat.

8. A floor covering comprising an impregnated felt base, a first imperforate coating of a mixture of nitrocellulose and a softening medium on the opposite faces of said base, a coating of paint on said first coating, and a second and transparent coating of nitrocellulose on the outer surface of said paint coat.

9. The process of making floor coverings which comprises treating a felt base which has been saturated throughout by coating it with a first coating of a solution of a cellulose ester, drying said coating, applying to said dried surface a coat of paint, and applying a second and transparent coating of a solution of a cellulose ester.

10. The process of making floor coverings which comprises treating a felt base, which has been saturated throughout, by coating it with a first coating solution of a cellulose ester, drying said solution, applying to said dried surface a coat of paint, and applying to said paint coat a second and transparent coating of a mixture in solution of a cellulose ester and a softening medium.

11. The process of making floor coverings which comprises coating an impregnated felt base with a coating solution of a cellulose ester, drying said solution, applying to said dried surface a coat of paint, and applying to said paint coat a second and transparent coating of a mixture in solution of 10 parts by weight of a cellulose ester, 90 parts of a solvent therefor, and 10 parts of a softening medium.

12. The process of making floor coverings which comprises coating an impregnated felt base with a solution of a cellulose ester, which solution contains approximately 12 parts by weight of a cellulose ester and 88 parts of solvent therefor, drying said solution, applying to said dried surface a coat of paint, and applying to said paint coat a second and transparent coating of a mixture in solution of 12 parts by weight of a cellulose ester, 90 parts of

a solvent therefor, and 10 parts of a softening medium.

13. The process of making floor coverings which comprises coating an impregnated felt base with a solution of a cellulose ester, 70 which solution contains approximately 12 parts by weight of a cellulose ester, 88 parts of solvent therefor and 10 parts of a softening medium, drying said solution, applying to said dried surface a coat of paint, and applying to said paint coat a second and transparent coating of a mixture in solution of 10 parts by weight of a cellulose ester, 90 parts of a solvent therefor, and 10 parts of a softening medium.

14. The process of making floor coverings which comprises treating a felt base, which has been saturated throughout, by coating it with a first coating of a solution of a cellulose ester, drying said coating, applying to said dried surface a coat of paint, and applying a second and transparent coating of a solution of a cellulose ester.

15. The process of making floor coverings which comprises treating a felt base, which has been saturated throughout, by coating it with a first coating of a solution of nitrocellulose, drying said coating, applying to said dried surface a coat of paint, and applying a second and transparent 95 coating of a solution of nitrocellulose.

16. The process of making floor coverings which comprises treating a felt base, which has been saturated throughout, by coating it with a first coating solution of nitrocellulose, drying said solution, applying to said dried surface a coat of paint, and applying to said paint coat a second and transparent coating of a mixture in 105 solution of nitrocellulose and a softening medium.

17. The process of making floor coverings which comprises coating an impregnated felt base with a coating solution of nitrocellulose, drying said solution, applying to 110 said dried surface a coat of paint, and applying to said paint coat a second and transparent coating of a mixture in solution of 10 parts by weight of nitrocellulose, 90 parts of a solvent therefor, and 10 parts 115 of a softening medium.

18. The process of making floor coverings which comprises coating an impregnated felt base with a solution of nitrocellulose, which solution contains approximately 12 120 parts by weight of nitrocellulose and 88 parts of solvent therefor, drying said solution, applying to said dried surface a coat of paint, and applying to said paint coat a second and transparent coating of a mixture in solution of 10 parts by weight of nitrocellulose, 90 parts of a solvent therefor, and 10 parts of a softening medium.

19. The process of making floor coverings which comprises coating an impregnated 130

felt base with a solution of nitrocellulose, which solution contains approximately 12 parts by weight of nitrocellulose, 88 parts of solvent therefor and 12 parts of a softening medium, drying said solution, applying to said dried surface a coat of paint, and applying to said paint coat a second and transparent coating of a mixture in solution of 10 parts by weight of nitrocellulose, 10 90 parts of a solvent therefor, and 10 parts of softening medium.

20. The process of making floor coverings which comprises treating a felt base, which has been saturated throughout, by coating 15 it with a first coating of a solution of nitrocellulose, drying said coating, applying to said dried surface a coat of paint, and applying a second and transparent coating of a solution of nitrocellulose.

21. A smooth surface floor covering comprising a porous base saturated throughout with an impregnating material and dried, a first imperforate coating of a cellulose ester on said base, a coating of paint on said cellulose ester, and a second and transparent 25 coating of a cellulose ester material on the outer surface of said paint coat.

22. A smooth surface floor covering comprising a porous fibrous base saturated throughout with an impregnating material 30 and dried, a first imperforate coating of a cellulose ester material on said paint, a coating of paint on said first coat, and a second and transparent coating of a cellulose ester material on the outer surface of said paint coat.

In testimony whereof I affix my signature.  
CALEB MARSHALL TAYLOR.